

# UNITED STATES PATENT OFFICE.

JOSEPH F. BEATTIE, OF HURLEY, NEW MEXICO.

## MOTOR FUEL.

No Drawing.

Application filed November 11, 1925. Serial No. 68,470.

The present invention relates to an improved motor fuel, for use in internal combustion engines, such as ordinary automobile engines, and is preferably used with a jet carburetor, although it can be employed with other kinds of carburetors.

In accordance with the present invention, I dissolve a small amount of paraffin wax in gasoline, the amount of paraffin wax being variable within rather wide limits. In the preferred form of the invention I preferably employ about .7% by weight, although I have used various quantities between .35% and 2.1%, with satisfactory results. In the preferred form of the process, I preferably mix one pound of paraffin with each twenty gallons of the gasoline, and the fuel is readily handled by an ordinary carburetor without any difficulty.

By the use of my fuel, accumulations of carbon in the cylinders of the engine are readily removed, and the formation of further deposits of carbon is largely prevented. In addition the lubrication of the piston in the cylinder is greatly facilitated, on account of the lubricating qualities of the paraffin wax itself. By the use of my fuel, the consumption of oil (engine lubricating oil) has been cut down.

The use of this fuel has given particu-

larly good results in high altitudes, such as one to two miles, although it will be understood that the fuel can be used anywhere.

A particular advantage of my fuel is that the engine does not knock near as badly as with ordinary straight run gasoline. By the use of my gasoline, I secure about 18 to 20% more mileage per gallon, than with ordinary straight run gasoline, such as that obtained from the California and Texas oils. The engine runs more smoothly with my product, and shows better acceleration. While I have used Texas and California gasolines, in combination with paraffin wax, the invention is not restricted to the use of this particular kind of gasoline.

I claim:—

1. A motor fuel comprising gasoline carrying a small percentage of paraffin wax in solution therein.
2. A motor fuel comprising gasoline carrying about .35 to 2.1% of paraffin wax in solution therein.
3. A motor fuel comprising gasoline carrying about .7% of paraffin wax in solution therein.

In testimony whereof I affix my signature.

JOSEPH F. BEATTIE.